

# UNITED STATES PATENT OFFICE.

SAMUEL KRAUS, OF NEW YORK, N. Y., ASSIGNOR TO THE EAGLE PENCIL COMPANY, OF SAME PLACE.

## COLORED LEAD FOR PENCILS.

SPECIFICATION forming part of Letters Patent No. 316,373, dated April 21, 1885.

Application filed March 5, 1885. (No specimens.)

*To all whom it may concern:*

Be it known that I, SAMUEL KRAUS, of the city, county, and State of New York, have invented a certain new and useful Improvement 5 in Colored Leads for Pencils, &c., of which the following is a specification.

My invention has relation to what are commonly known in the art of lead-pencil-making as "colored" leads or "crayon" leads— 10 that is to say, blue, white, red, green leads, and the like, as contradistinguished from the ordinary graphite pencil-lead.

In making colored lead heretofore it has been the practice to mold or press it from a 15 composition consisting of the color—red, blue, or the like—a base—such as kaolin—and a binding medium or gum—such, for instance, as gum-tragacanth. This process of manufacture is not only tedious and expensive, but is 20 uncertain to some extent in its results, and often results in the production of an inferior article. The composition, owing to the gum which it contains, cannot be baked, but must simply be dried, and the gum affects often 25 times the quality of the article.

It is the object of my invention to remove these obstacles and to produce a colored lead which can be made as easily and inexpensively as the ordinary graphite pencil-lead, and 30 which shall possess equal efficiency. To obtain this result it is requisite to bake the colored composition lead; but to do this it is indispensable that the gum ordinarily used should be dispensed with, because the effect of 35 the baking operation would be to entirely burn and destroy it; and it is also requisite to employ colors which will withstand without deterioration the heat requisite for the baking operation. Among such colors, which 40 may be named by way of example, are iron-red, ultramarine, burnt sienna, Indian red, chrome and mineral yellow, (I use a mixture of the two for the production of a yellow, inasmuch as the chrome-yellow alone will not 45 withstand so well the heat,) and what is known as "Victoria," "permanent," or "lump" green. I use as a base, preferably, a mixture of talc or soapstone and potter's clay, and to 50 this base I add the requisite quantity of color of the shade required, together with a little

graphite, if it be required to modify or darken the shade.

For what is known in the trade as a "medium soft lead," the ingredients may be taken in about the following proportions: coloring-matter, (of the character above specified,) ten pounds; talc or soapstone, five pounds; potter's clay, ten pounds. I here remark that by increasing or decreasing the proportion of potter's clay the lead produced will be rendered proportionately harder or softer. These ingredients are mixed with water to a paste, and are then ground, so as to be finely reduced and intimately mixed and brought to the condition of a smooth homogeneous paste. Then 65 by means of a press—such as employed in the manufacture of pencil-leads and well known to those skilled in the art to which my invention pertains—the composition is molded or brought to the shape of a pencil-lead. In 70 this condition it is allowed to thoroughly dry. After drying it is baked. For this purpose the furnace or baking chamber is preliminarily raised to about a bright-red heat, the dried colored lead is placed therein and allowed to 75 remain about ten minutes, or until it is heated to a dull-red heat. It is then withdrawn and allowed to cool. In this condition it has the characteristics of a slate-pencil, and is still 80 unfit for use as a colored pencil-lead. The final operation is to boil it in fat or oil—such, for instance, as stearine, which I find on the whole productive of the best results. It is immersed in the boiling stearine, and is there allowed to remain for twenty minutes, or thereabout. This last-named operation changes 85 the characteristics of the article and converts it into a pencil-lead which is quite as good as and in some respects superior to the ordinary colored lead or crayon hitherto made.

One great advantage is, that my colored lead can be made of as small diameter as the ordinary graphite pencil-lead without any more danger of breaking when in use, which is not feasible with colored leads as ordinarily manufactured. Another advantage is, that marks made by it can be erased without smearing or soiling the paper, which is not the case with ordinary colored leads.

Having described my improvement and the 100

best way now known to me of carrying the same into effect, I wish it to be understood that I do not restrict myself to the particular details hereinbefore set forth illustrative of the improvement, for the same can be considerably varied without departure from the principle of the invention; but

What I consider to be new and of my own invention is—

10 1. A colored pencil-lead made and possessing the characteristics substantially as hereinbefore set forth.

2. The improvement in the manufacture of colored pencil-leads, consisting in molding the same from a composition of the kind hereinbefore described, drying and baking the molded article, and subsequently boiling it in fat or oil, substantially as set forth.

In testimony whereof I have hereunto set my hand this 4th day of March, 1885.

SAMUEL KRAUS.

Witnesses:

JOE W. SWAINE,

LEOPOLD ANSBACHER.